

# United States Patent

[19]

Conner

[11] 3,895,907

[45] July 22, 1975

[54] **TURNBULL'S BLUE SINGLE BATH  
MINERAL DYEING PROCESS  
(FERRI-ZIRC) FOR CELLULOSIC  
TEXTILES**

[75] Inventor: **Charles James Conner**, New Orleans, La.

[73] Assignee: **The United States of America as represented by the Secretary of Agriculture**, Washington, D.C.

[22] Filed: **Oct. 10, 1973**

[21] Appl. No.: **404,974**

[52] U.S. Cl..... **8/52; 8/17**

[51] Int. Cl..... **D06p 3/60**

[58] Field of Search..... **8/52, 17, 30**

[56] **References Cited**

UNITED STATES PATENTS

|           |         |              |      |
|-----------|---------|--------------|------|
| 1,661,606 | 3/1928  | Escaich..... | 8/52 |
| 1,686,540 | 10/1928 | White .....  | 8/52 |
| 2,214,845 | 9/1940  | Wells .....  | 8/52 |
| 2,923,592 | 2/1960  | Croslan..... | 8/52 |
| 3,671,178 | 6/1972  | Conner ..... | 8/52 |
| 3,702,753 | 11/1972 | Conner ..... | 8/52 |
| 3,705,004 | 12/1972 | Conner ..... | 8/52 |
| 3,768,965 | 10/1973 | Conner ..... | 8/52 |
| 3,779,702 | 12/1973 | Conner ..... | 8/52 |

3,791,786 2/1974 Conner .....

3,794,466 2/1974 Conner .....

8/52

8/52

## OTHER PUBLICATIONS

American Dyestuff Reporter, March 1974, pp. 37-45.

Textile Research Journal, April 1964, pp. 347-357.

Textile Research Journal, February 1967, pp. 94-102.

"One-Bath Zirchrome Chloride Fungicide and Dye" by C. J. Conner, et al.

Primary Examiner—Benjamin R. Padgett

Assistant Examiner—D. P. Walsh

Attorney, Agent, or Firm—M. Howard Silverstein; Max D. Hensley

[57]

## ABSTRACT

Certain inhibited reducing agents are combined in a single bath with a ferric salt and an alkali metal ferricyanide, which is activated by heat decomposition of the inhibited reducers, to cause reduction of the ferric salt to the ferrous state on the cellulosic, in contact with the ferricyanide, thereby producing Turnbull's Blue in the cellulosic textile. A zirconium salt is used in the bath to lock the dye to the cellulosic. The resulting uniform pure blue mineral dyeing of cellulose by this single bath process has been defined as the FERRI-ZIRC BLUE PROCESS.

**8 Claims, No Drawings**

TURNBULL'S BLUE SINGLE BATH MINERAL  
DYEING PROCESS (FERRI-ZIRC) FOR  
CELLULOSIC TEXTILES

A non-exclusive, irrevocable, royalty-free license in the invention herein described throughout the world for all purposes of the United States Government, with the power to grant sublicenses for such purposes, is hereby granted to the Government of the United States of America.

This invention relates to mineral dyeing of cellulosic textiles. More specifically, this invention relates to a single-bath textile dyeing process which utilizes a ferric salt, and ammonium sulphite of ammonium oxalate as an inhibited reducing agent, which are combined without reaction with an alkali metal ferricyanide and zirconyl ammonium carbonate to produce a stable single bath solution. The solution thus prepared remains clear as long as it remains alkaline due to the presence of ammonium ions. When the prescribed conditions are adhered to a Turnbull's Blue coloration is imparted to cellulosic textiles. The finished product contains the blue coloration combined with zirconia from heat decomposition of the zirconyl ammonium carbonate, causing the Turnbull's Blue-zirconia deposit to lock onto the cellulosic textile, thus making the blue pigment significantly more resistant to alkalis than it would be if the zirconyl ammonium carbonate were not included in the formulation.

The main object of this invention is to provide a single-bath system for dyeing Turnbull's Blue color shades by a simple pad (wetting and squeezing out excess bath), dry and cure procedure, followed by wash and dry to remove byproducts.

A second object of this invention is to provide an attractive and appealing color shade for the textile dyer, by shorter processing and requiring less mill equipment.

A third object of this invention is to provide a single-bath system for Turnbull's Blue mineral dyeing that can be finished with a paraffin-ammonium stearate wax, requiring no after-rinse with aluminum formo-acetate to neutralize the residual stearic acid. The hydrous zirconia in the invention dyeing reacts with and neutralizes the stearic acid, without an added step.

The utility of this invention, therefore, is obviously in the field of mineral dyeings of cellulosic textiles to obtain attractive and specific blue color shades in finished goods such as curtains, umbrellas, tents, sails, awnings, canvas shoes, upholstery, etc.

The prior art teaches that water-soluble ferrous salts react with water soluble alkali metal ferricyanides to produce an insoluble blue dye pigment of ferrous ferricyanide known as Turnbull's Blue. It has also been known from the prior art that cellulosics can be wetted with a ferrous salt, and then with a solution of alkali metal ferricyanide, using two separate baths, to produce ferrous ferricyanide by double decomposition.

Now, this writer has unexpectedly discovered what is disclosed in the process of this invention. The present invention provides a unique single-bath system where a ferric salt and ammonia inhibited reducing agents; i.e., ammonium oxalate and ammonium sulfite, are combined together without reaction—with an alkali metal ferricyanide and zirconyl ammonium carbonate—to produce a stable single bath, clear, system as long as it remains alkaline from the presence of ammonium ions. In this state it may be applied to cellu-

losic textiles. When the wet impregnated textile is heated up to about from 150° to 160°C. the ammonium salts are decomposed, ammonia leaves the system, and the oxalate and sulfite ions remaining, are capable of reducing the ferric salt to the ferrous state, when it reacts with the ferricyanide in the cellulosic textile, to produce ferrous ferricyanide (Turnbull's Blue). During the same heat cure the zirconyl ammonium carbonate decomposes to liberate ammonia and carbon dioxide and produce hydrous zirconia, which is deposited as a "lake" with the Turnbull's Blue dye pigment. Beautiful pure blue mineral dyeings are produced in the cellulose by simply wetting and heating the wetted cellulosic to develop the dye.

EQUATIONS PERTINENT TO THIS INVENTION



\*R represents either sodium or potassium.



SUMMARY OF THE INVENTION

In brief the present invention can best be described as a plurality of mineral dye baths as well as a mineral dyeing process for cellulosic textiles. One of the preferred embodiments would be described as a dye bath for imparting to cellulosic textiles a durable-to-water-washing Turnbull's Blue coloration, the said dye bath containing...

about from 1 to 5 parts by weight of sodium or potassium ferricyanide,

about from 2 to 5 parts by weight of ammonium oxalate monohydrate,

about from 1 to 5 parts by weight of ferric sulphate, about from 5 to 10 parts by weight of zirconyl ammonium carbonate solution (aqueous 10 percent ZrO<sub>2</sub>), and

about 60 to 85 parts by weight of water.

Another of the preferred embodiments of this invention would be described as a mineral dyeing process to impart durable-to-water-washing Turnbull's Blue coloration to cellulosic textiles, the process comprising...

a. impregnating a cellulosic textile with an aqueous solution containing...

about from 1 to 5 parts by weight of potassium ferricyanide,

about from 2 to 5 parts by weight of ammonium oxalate monohydrate,

about from 1 to 5 parts by weight of ferric sulphate,

- about from 5 to 10 parts by weight of ammonium sulphite monohydrate,  
about from 1 to 5 parts by weight of monoethanolamine, and  
about from 5 to 10 parts by weight of zirconyl ammonium carbonate solution (aqueous 10 percent  $ZrO_2$ );  
b. removing the excess solution to obtain a wet pickup of about 70-80 percent,  
c. drying the wet impregnated textile for about 2 minutes at about  $120^\circ$  to  $130^\circ C$ ., and  
d. curing the textile for about 2 minutes at about from  $150^\circ$  to  $155^\circ C$ .

The following examples are provided to illustrate the preferred embodiments of the invention, and should not be construed as limiting the invention in any manner whatever. The various formulations and techniques were employed with paper, wood, and other textiles having partial quantities of cellulose.

#### EXAMPLE 1

5 Grams of potassium ferricyanide, 20 grams of water and 2 grams of ferric sulphate were dissolved together in 43 grams of water (distilled). To this was added 10 grams of ammonium sulphite (monohydrate) crystals. Upon stirring, a clear brown colored bath resulted. No Turnbull's Blue precipitated, and the sulfite reducer was inhibited by the ammonium (alkaline) ion. This bath was capable of dyeing a pure blue by heat (150°C.) decomposition on a cellulosic.

5

15

20

25

30

|                                                                         |
|-------------------------------------------------------------------------|
| 1.00 to 5.00 grams Sodium or Potassium Ferricyanide Crystals            |
| 60.00 to 85.00 grams Water (distilled or soft)                          |
| 2.00 to 5.00 grams Ammonium Oxalate Crystals (monohydrate)              |
| 1.00 to 5.00 grams Ferric Sulphate ( $Fe_2(SO_4)_3 \times H_2O$ )       |
| 5.00 to 10.00 grams Zirconyl Ammonium Carbonate Solution (10% $ZrO_2$ ) |
| 5.00 to 10.00 grams Ammonium Sulfite Crystals (monohydrate)             |
| 1.00 to 5.00 grams Monoethanolamine                                     |

100.0 grams Clear Greenish-Black Single Bath (Ferri-Zirc)

#### EXAMPLE 2

The bath from Example 1 was used to wet a  $6 \times 3$  inch piece of scoured canvas duck, the excess being blotted off. The wet treated duck was dried at  $120^\circ$  for 2 minutes and then cured at  $150^\circ C$ . for 2 minutes. The fabric was dyed deep pure Turnbull's Blue. It was washed for 2 minutes in hot running tap water and oven dried at  $130^\circ C$ . for 2 minutes. The fabric remained uniformly dyed a pure deep Turnbull's Blue.

45

50

#### EXAMPLE 3

One gram of potassium ferricyanide, 1 gram of ferric sulphate, and 1 gram of ammonium oxalate were dissolved together in 27 grams of distilled water. A greenish-yellow single bath resulted, all ingredients being soluble. On wetting a piece of scoured duck (2x4 inches) with the bath and then heating it to  $150^\circ C$ . for 2 minutes, a deposit of Turnbull's Blue was produced, dyeing the fabric pure deep Turnbull's Blue, and showing ammonium oxalate to be a suitable inhibited reducer in the bath. Due to lack of sufficient ammonium ion alkalinity, the bath stability was poor, and some blue precipitations occurred in the bath after 10 minutes. (5993-121)

55

60

65

#### EXAMPLE 4

The following formulation utilizes both ammonium oxalate and ammonium sulfite for increased bath alkalinity and stability:

|                                          |
|------------------------------------------|
| 3.0 grams distilled water                |
| 80.0 grams distilled water               |
| 3.0 grams ferric sulphate                |
| 3.0 grams ammonium oxalate               |
| 9.0 grams ammonium sulfite (monohydrate) |
| 2.0 grams monoethanolamine               |

100.0 grams Clear Greenish-Black Bath

The addition of a small amount of monoethanolamine gives an increased alkaline stability and bath stability.

#### EXAMPLE 5

Scoured duck and paper towels were wetted with the bath from Example 4, and heated to  $155^\circ C/2$  minutes. Uniform, pure blue deep Turnbull's Blue dye shades were produced, which were stable to hot tap water washing ( $55^\circ C/2$  minutes).

#### EXAMPLE 6

The incorporation of zirconyl ammonium carbonate (10 percent  $ZrO_2$ ) into Example 6, produces a brighter pure blue color shade through "lake" formation of the Turnbull's Blue with zirconia. The following formulation variations were prepared and successfully evaluated:

|                                                                         |
|-------------------------------------------------------------------------|
| 1.00 to 5.00 grams Sodium or Potassium Ferricyanide Crystals            |
| 60.00 to 85.00 grams Water (distilled or soft)                          |
| 2.00 to 5.00 grams Ammonium Oxalate Crystals (monohydrate)              |
| 1.00 to 5.00 grams Ferric Sulphate ( $Fe_2(SO_4)_3 \times H_2O$ )       |
| 5.00 to 10.00 grams Zirconyl Ammonium Carbonate Solution (10% $ZrO_2$ ) |
| 5.00 to 10.00 grams Ammonium Sulfite Crystals (monohydrate)             |
| 1.00 to 5.00 grams Monoethanolamine                                     |

100.0 grams Clear Greenish-Black Single Bath (Ferri-Zirc)

#### EXAMPLE 7

All of the above bath variations could be used successfully to produce single bath Turnbull's Blue color shades with heat curings at  $150^\circ$  to  $155^\circ C$  for 1 to 3 minutes, using scoured duck or paper.

#### EXAMPLE 8

The following bath formulation gave excellent color shades, on duck, and showed a bath stability of 10 hours: (6519-82)

|                                                                 |
|-----------------------------------------------------------------|
| 3.00 grams Potassium Ferricyanide Crystals                      |
| 70.00 grams Water                                               |
| 3.00 grams Ammonium oxalate                                     |
| 3.00 grams Ferric Sulphate                                      |
| 10.00 grams Zirconyl Ammonium Carbonate Solution (10% $ZrO_2$ ) |
| 9.00 grams Ammonium Sulfite (monohydrate)                       |
| 2.00 grams monoethanolamine                                     |

#### EXAMPLE 9

Samples of scoured duck were wetted with the bath from Example 8 and oven dried at  $120^\circ C$ . for 2 minutes, followed by oven curing at  $150^\circ C$ . for 2 minutes. Excellent results were obtained. Other samples were dried at  $130^\circ C$ . for 1 minute, followed by oven curing

at 155°C. for 1 minute. Excellent results were again obtained. Evaluations indicate that predrying produces a uniform deposit of bath solids and reaching a temperature of 150°C. or higher is only required to effect decomposition of all ammonium salts.

#### EXAMPLE 10

The amount of monoethanolamine in Example 8, was varied up to 5 grams, and the bath stability observed. With 5 grams of this amine stabilizer, the life of the bath was increased to 48 hours.

#### EXAMPLE 11

The incorporation of zirconyl ammonium carbonate in the dye also results in a Turnbull's Blue zirconia dyeing on cellulosics, which is much more resistant to alkaline water washing than dyeing from the dye bath without zirconyl ammonium carbonate. Two baths were prepared as follows:

##### A

|                                                                |
|----------------------------------------------------------------|
| 3.0 gram Potassium or Sodium Ferricyanide                      |
| 70.0 gram Water (soft or distilled)                            |
| 3.0 grams Ammonium Oxalate                                     |
| 3.0 grams Ferric Sulphate                                      |
| 10.0 grams Zirconyl Ammonium Carbonate (10% ZrO <sub>2</sub> ) |
| 9.0 grams ammonium Sulphite                                    |
| 2.0 grams Monoethanolamine                                     |
| 100.0 grams Bath A (with Zr)                                   |

##### B

|                                           |
|-------------------------------------------|
| 3.0 gram Potassium or Sodium Ferricyanide |
| 80.0 gram Water (soft or distilled)       |
| 3.0 gram Ammonium Oxalate                 |
| 3.0 gram Ferric Sulphate                  |
| 9.0 gram Amminium Sulphite                |
| 2.0 gram Monoethanolamine                 |
| 100.0 gram Bath B (No Zr)                 |

Fabric samples were separately wetted in A and B, blotted free of excess, and dried 120°-130°C/2 minutes, followed by oven curing at 150°-155°C/2 minutes. The cured A and B fabrics were both dyed pure blue. When washed for 10 minutes in alkaline tap water (pH10.0), the A sample remained pure blue (with Zr) while, the B sample (no Zr) showed a blue and brown discolored appearance, due to alkaline hydrolysis of the ferrous ferricyanide (Turnbull's Blue).

#### EXAMPLE 12

The fabric sample A from Example 11, after cure and wash, was wetted with a 7 percent paraffin emulsion (paraffin-ammonium stearate type), squeezed free of excess liquid, and oven dried at 120°-130°C. for 2 minutes, followed by raising the temperature to 150°C. for 1 minute. The cooled paraffin finished sample was deep blue in color, and water repellent (spray rated 90-100).

I claim:

1. A mineral dyeing process for imparting a Turnbull's Blue coloration to cellulosic textiles, the process consisting of impregnating a cellulosic textile with an aqueous solution containing an inhibited reducing agent, ferric salt, and alkali metal ferricyanide, and zirconyl ammonium carbonate, then curing the impregnated cellulosic textile.

2. A mineral dyeing process to impart durable-to-water washing Turnbull's Blue coloration to cellulosic textiles, the process comprising . . .

- a. impregnating a cellulosic textile with an aqueous solution containing . . .
- about from 1 to 5 parts by weight of sodium ferricyanide,
- about from 2 to 5 parts by weight of ammonium oxalate monohydrate,
- about from 1 to 5 parts by weight of ferric sulphate,
- about from 1 to 10 parts by weight of ammonium sulphite monohydrate,
- about from 1 to 5 parts by weight of monoethanolamine, and
- about from 5 to 10 parts by weight of zirconyl ammonium carbonate solution (aqueous 10 percent ZrO<sub>2</sub>);

- b. removing the excess solution to obtain a wet pickup of about 70-80 percent,
- c. drying the wet impregnated textile for about 2 minutes at about 120° to 130°C., and
- d. curing the textile for about 2 minutes at about from 150° to 155°C.

3. A mineral dyeing process to impart durable-to-water washing Turnbull's Blue coloration to cellulosic textiles, the process comprising . . .

- a. impregnating a cellulosic textile with an aqueous solution containing . . .
- about from 1 to 5 parts by weight of potassium ferricyanide,
- about from 2 to 5 parts by weight of ammonium oxalate monohydrate,
- about from 1 to 5 parts by weight of ferric sulphate,
- about from 5 to 10 parts by weight of ammonium sulphite monohydrate,
- about from 1 to 5 parts by weight of monoethanolamine, and
- about from 5 to 10 parts by weight of zirconyl ammonium carbonate solution (aqueous 10 percent ZrO<sub>2</sub>);

- b. removing the excess solution to obtain a wet pickup of about 70-80 percent,
- c. drying the wet impregnated textile for about 2 minutes at about 120° to 130°C., and
- d. curing the textile for about 2 minutes at about from 150° to 155°C.

4. A dye bath for imparting to cellulosic textiles a durable-to-water-washing Turnbull's Blue coloration, the said dye bath containing . . .

- about from 1 to 5 parts by weight of sodium ferricyanide,
- about from 2 to 5 parts by weight of ammonium oxalate monohydrate,
- about from 1 to 5 parts by weight of ferric sulphate,
- about from 5 to 10 parts by weight of ammonium sulphite monohydrate,
- about from 1 to 5 parts by weight of monoethanolamine,
- about from 50 to 10 parts by weight of zirconyl ammonium carbonate solution (aqueous 10 percent ZrO<sub>2</sub>), and
- about from 60 to 85 parts by weight of water.

5. A dye bath for imparting to cellulosic textiles a durable-to-water-washing Turnbull's Blue coloration, the said dye bath containing . . .

- about from 1 to 5 parts by weight of potassium ferricyanide,

about from 2 to 5 parts by weight of ammonium oxalate monohydrate,  
 about from 1 to 5 parts by weight of ferric sulphate,  
 about from 5 to 10 parts by weight of ammonium sulphite monohydrate,  
 about from 1 to 5 parts by weight of monoethanolamine,  
 about from 5 to 10 parts by weight of zirconyl ammonium carbonate solution (aqueous 10 percent  $ZrO_2$ ), and  
 about from 60 to 85 parts by weight of water.

6. A dye bath for imparting to cellulosic textiles a Turnbull's Blue coloration, the dye bath containing.

5 parts by weight of potassium ferricyanide,  
 2 parts by weight of ferric sulphate,  
 10 parts by weight of ammonium sulphite monohydrate, and  
 20 parts by weight of water . . . to give a clear brown solution.

15  
20

7. A dye bath for imparting to cellulosic textiles a Turnbull's Blue coloration, the dye bath containing.

1 part by weight of potassium ferricyanide,  
 1 part by weight of ferric sulphate,  
 1 part by weight of ammonium oxalate, and  
 27 parts by weight of water . . . to give a greenish-yellow solution.

8. A dye bath for imparting to cellulosic textiles a Turnbull's Blue coloration, the dye bath containing.

3 parts by weight of sodium ferricyanide,  
 3 parts by weight of ferric sulphate,  
 3 parts by weight of ammonium oxalate,  
 9 parts by weight of ammonium sulfite monohydrate,  
 2 parts by weight of monoethanolamine, and  
 80 parts by weight of water . . . to give a clear greenish-black solution.

\* \* \* \* \*

25

30

35

40

45

50

55

60

65